

L. F. HAWLEY.

PROCESS FOR PRODUCING DENSE ABSORBENT CHARCOAL.

APPLICATION FILED APR. 3, 1919.

1,385,826.

Patented July 26, 1921.



# UNITED STATES PATENT OFFICE.

LEE F. HAWLEY, OF MADISON, WISCONSIN, ASSIGNOR TO UNITED STATES OF AMERICA.

## PROCESS FOR PRODUCING DENSE ABSORBENT CHARCOAL.

1,385,826.

Specification of Letters Patent.

Patented July 26, 1921.

Application filed April 3, 1919. Serial No. 287,315.

To all whom it may concern:

Be it known that I, LEE F. HAWLEY, a citizen of the United States, residing at Madison, in the county of Dane and State of Wisconsin, have invented certain new and useful Improvements in Processes for Producing Dense Absorbent Charcoal, of which the following is a specification.

This invention relates to an improved process of making a very dense and homogeneous charcoal from wood or similar vegetable material.

The product of this invention may be utilized for the absorption of gases.

Ordinarily, the distillation of wood in the manufacture of charcoal has provided a light porous charcoal. The density of the resultant charcoal has always varied with the type of wood used, a very heavy dense wood providing a charcoal normally more dense than that made from the lighter types of wood. As a result of the present invention it is now possible to obtain from the lighter types of wood a charcoal much more dense than that heretofore obtained from the heaviest woods.

The present invention makes it possible to provide a charcoal having a density of at least .95 when an ordinary light wood is used, and a density of at least 1.05 when this same wood has been given a preliminary hydrolyzing treatment.

The process comprises the comminution of the wood to saw-dust or wood flour and the compression of this material in molds into solid blocks. These blocks are formed under a pressure of at least 30,000 pounds per square inch. The blocks thus formed are then distilled and at the same time subjected to a constant and directly applied mechanical compression of at least 100 pounds per square inch. The unusually high compression during distillation produces the dense product desired. This remarkable result is effected by the mechanical compression during distillation and is due in part to the fact that there is a stage in the distillation of the blocks of compressed wood, just as the wood is decomposing into charcoal, when the charcoal is slightly plastic and a sufficiently great pressure therefore closes the pores and interstices thereof and forms a homogeneous dense charcoal.

The detailed steps in the process may be carried out as described hereinafter. Any

ordinary wood, such as birch, maple, or pine is cut or ground to a finely divided condition like saw-dust or wood flour. This comminuted material is then compressed in any suitable mold, not shown, under a pressure of at least fifteen tons, 30,000 pounds, to the square inch, thus forming a solid block of wood having a density of about 1.10. These blocks or briquets are preferably circular in cross section and with smooth flat ends. A desirable size is one having a diameter of four inches and a thickness of three inches. The briquets so made are then placed face to face in a metal tube, having a diameter slightly greater than that of the briquets. If placed face to face within the tube the briquets form a rod of compressed wood. However, if it is desired to space the briquets apart, either to permit the passage of gases or to preserve the identity of the briquets, this may be done by introducing between the briquets thin sheets of metal of the same diameter of the briquets, or smaller than the bore of the tube. Endwise pressure is applied to the column of briquets. This pressure is constant and may amount to from 100 to 250 pounds per square inch. The tube and its contents are subjected to a distillation temperature of at least 300° C. during which treatment the pressure is continuously maintained. The plastic stage of the material during distillation covers only a small range of temperatures, from about 280° C.-300° C., and if the distillation temperature is carried much above this point it is not necessary, and often not desirable, to apply extreme pressure during the last stage of distillation.

Different pressure for the process may necessarily be adopted for varied conditions. For instance, with a pressure of 30,000 pounds per inch on the briquets used prior to distillation a pressure of 250 pounds per square inch is necessary during distillation to secure best results, but with a pressure of 60,000 pounds per square inch used prior to distillation only 100 pounds is necessary during distillation. Likewise, a pressure of 250 pounds per square inch maintained throughout the distillation would be too high, and this sustained pressure would negative the advantages obtained by its application early in the distillation treatment, the charcoal being shattered and rendered useless. On the other hand, if such a high

pressure be used only during the first part of the distillation the very best results may be obtained.

Volatile products of distillation consisting of tar, pyroligneous acid and gases can be trapped and used as desired as in the usual distillation of wood.

The same unusual results and dense charcoal may be obtained by utilizing a hydrolyzed wood product as the material for the briquets. In the process using hydrolyzed wood the comminuted wood is treated with dilute acid, preferably sulfuric acid, and high pressure steam, about 100 pounds per square inch, the water, sugar and other soluble materials are removed, the remaining material dried and briquetted and distilled as before. The resulting wood products remaining after the extraction process is produced in large and commercial quantities in the manufacturing plants engaged in the manufacture of ethyl alcohol from waste wood. If this residue is briquetted and distilled under the conditions of this invention the resultant charcoal is denser, about 1.05, than that obtained directly from wood by the process.

The process may be conducted in any suitable form of apparatus capable of performing the steps specified. The briquets may be formed in any suitable machine. The combined distillation and compression steps require a rather unusual type of structures, a suitable form of which is illustrated in the accompanying drawing, in which—

Figure 1 is a vertical sectional elevation illustrating the compression tube mounted in the distilling chamber,

Fig. 2 is a sectional view taken on the line 2—2 of Fig. 1,

Fig. 3 is a view taken on the line 3—3 of Fig. 1 looking in the direction of the arrow.

Referring in detail to the drawing 1 indicates the masonry of the end walls of a distillation furnace, 2 indicates the side walls and 3 the top of the furnace. The necessary strength for the structure is made certain by the liberal use of metal reinforcing where necessary. Each of the end walls have two parallel I-beams 4 positioned vertically and mounted in a concrete base 5. Suitable braces 6 are provided to strengthen the lower ends of the beams 4 and tie-rods 7 extend from the upper part of the beams 4 to further brace the structure. The furnace is long and narrow and is adapted to be heated by any type of fuel. As illustrated, the furnace is constructed to use gas or oil as fuel. Adjacent the lower part of the side walls 2 and spaced along the sides of the same are a series of ports or openings 8 adapted to receive burner nozzles projecting from any suitable supply gas pipe or oil pipe. The flame and hot gases pass upward and

through the outlet openings 9 provided in the top 3.

The apparatus for compressing the briquets during distillation includes a cylindrical metal tube or pipe 10 extending longitudinally of the furnace and projecting beyond the end walls thereof. This pipe 10 is necessarily of heavy metal and in order to conform with the preferred type of briquet should have a 5 inch bore. The pipe 10 is positioned and securely held in one end wall 1 by the facing clamps 11 which are screw threaded on the pipe 10 and which clamp the wall and I-beams. The opposite end of the pipe 10 is securely positioned in the opposite end wall but is not clamped to the wall, thus allowing for longitudinal movement resulting from expansion or contraction of the tube during heating. Briquets are inserted into the bore of the pipe 10 through the end opening 12 which is provided with a cover plate 13 adapted to be bolted in place over the end of the pipe 10. Gases and vapors generated during the distillation pass upward and outwardly through the gas outlet passage 14 which is located between the cover plate 13 and the end of the furnace. Compression is effected by means of a plunger 15 having a drive rod 16 projecting beyond the packing gland 17 and extending to a suitable source of power indicated as a worm drive 18. The plunger 15 is adapted to move slowly within the pipe 10 and to compress the briquets during the heat treatment. The construction should provide for a drive rod such that the movement of the piston would be reciprocatory and not rotary as is shown diagrammatically on the drawings.

It is known that charcoal briquets have been made by compressing fibrous wood blocks and distilling the same under mechanically applied pressure. This pressure however was only sufficient to hold the blocks in close contact with each other. Certain disclosures have shown that it was old to exercise compression during distillation. The present invention provides for a change in the nature of the charcoal by tremendous pressure during distillation. The density of the resultant product is due to the combination of specific steps and pressures mentioned.

I claim—

1. The process of making charcoal having a specific gravity of at least .95 from wood which comprises comminuting wood, forming blocks of the comminuted wood, subjecting the blocks to a pressure of at least 30,000 pounds to the square inch, and distilling the blocks under a substantially constant directly applied mechanical pressure of at least 100 pounds per inch.

2. The process of making a dense and homogeneous charcoal which comprises

- 5 forming blocks by compressing comminuted wood, subjecting the blocks to a pressure of at least 30,000 pounds per square inch prior to distillation, and subjecting the 5 blocks to a combined distilling temperature and to a substantially constant directly applied mechanical pressure of at least 100 pounds per square inch.
- 10 3. The process of making charcoal having a specific gravity of at least .95 which comprises forming blocks by compressing comminuted wood, subjecting the blocks to a pressure of at least 30,000 pounds per square inch prior to heating them, subjecting the blocks to a combined heat treatment of 300° C. and to a directly applied mechanical pressure of at least 250 pounds per square inch, and subsequently maintaining the heat treatment and a lower pressure.
- 15 20 4. The process of making dense and homogeneous charcoal from wood which consists of comminuting wood, subjecting the comminuted wood to the action of sulfuric acid
- and steam under pressure, washing the material so treated, forming blocks by compressing the remaining comminuted material, subjecting the blocks to a pressure of at least 30,000 pounds per square inch prior to distillation, and subjecting the blocks to a combined distilling temperature and to a directly applied constant mechanical pressure of at least 100 pounds per square inch. 25
5. The process of making dense and homogeneous charcoal from wood which consists of comminuting the wood to be treated, hydrolyzing this material, forming blocks of the hydrolyzed material, subjecting the blocks to a pressure of at least 30,000 pounds to the square inch, and distilling the blocks under a substantially constant directly applied mechanical pressure of at least 100 pounds per inch. 30 35 40

In testimony whereof I have affixed my signature.

LEE F. HAWLEY.